

## UNITED STATES PATENT OFFICE

2,193,222

## VANADIUM STEEL ALLOY

Vere B. Browne, Brackenridge, Pa., assignor to  
Allegheny Steel Company, Brackenridge, Pa.,  
a corporation of Pennsylvania

No Drawing. Application January 2, 1930,  
Serial No. 417,927

4 Claims. (Cl. 75—128)

This invention relates to vanadium steel alloys and articles thereof having substantial immunity to intercrystalline disintegration or deterioration and more particularly to vanadium containing 5 chromium nickel steel alloys.

Chromium nickel steel alloys per se are well known and have high resistance to corrosion, except where the alloys are required to be heated to a temperature of around 500° to 900° C. without being subjected to a higher degree of heat, such as in welding. The consequences are that such alloys tend toward intercrystalline disintegration or deterioration unless annealed at temperatures several hundred degrees higher than 10 said 500°-900° C. temperature range. An annealing operation is not only inconvenient, and adds to the expense, but it distorts the alloy, especially if it has been provided with a particular shape or form so that further reshaping or 15 straightening steps are necessitated.

I have as an object of this present invention the provision of an alloy and article thereof obviating and overcoming the difficulties and disadvantages of known alloys and presenting novel 20 features and advantages peculiar to its own composition.

Another object of my invention is the provision of a chromium nickel steel alloy and article thereof containing vanadium, and having immunity to intercrystalline disintegration or 25 deterioration.

I accordingly utilize what I have found to be an excellent chromium nickel steel alloy and to it I add predetermined amounts of vanadium.

As the art of alloying various metals is known in the industry, such needs no detailed consideration here and the process or steps involved 30 form no part of this invention.

I may successfully use a chromium nickel steel 35 of the following range of composition:

|          | Per cent                     |
|----------|------------------------------|
| Chromium | 6-40                         |
| Nickel   | .5-25                        |
| Carbon   | 0-3                          |
| Iron     | Substantially entire balance |

It is not intended that the above represent the extremes of percentages as they are, rather, illustrative of conveniently obtainable compositions 50 to which vanadium may be added, as will be hereinafter explained more fully, and which, together with the vanadium, produces excellent and useful alloys having great advantages in the metallurgical, chemical, and physical fields.

Theoretically the chromium and nickel con-

tent may run from comparatively low percentages in the neighborhood of two or three percent to rather high percentages around 40, 50, 60, or even up to 80 or 90%. Such compositions all have certain advantages but in general may be 5 said to be of somewhat limited use in such connections as would be calculated to take advantage of the particular properties with which the different alloys were endowed by virtue of their composition.

The range of about 6-40% chromium and .5-25% nickel is more convenient and more widely applicable in the industry, the particular composition of 18% chromium and 8% nickel being a particularly well known and useful one. 10

To such alloys, as I have above outlined, I add, at suitable points in the production thereof, a predetermined amount of vanadium depending on the influence desired upon the ultimate product. The presence of vanadium seems to endow 15 the alloy with a particularly stubborn resistance to intercrystalline disintegration and deterioration and there is probably a combined chemical and physical interaction resulting partly in the formation of new chemical compounds 20 and partly in the formation of solid solutions. Whatever the actual or theoretical correlation 25 of the constituents, a new alloy is evolved by the invention having the advantages set forth and others besides from which useful articles in the 30 chemical, metallurgical and physical fields can be made.

The amount of vanadium added is predetermined according to the results preferred in the ultimate product and hence may range from 35 practically zero to several percent, or relatively large percentages, depending, too in a measure upon the intended use of the particular alloy and hence limited to some extent by the economics of the situation in question. A preferred 40 range extends from say .2% to 2 or 3%, but these figures are purely illustrative and variable according to circumstances.

Utilizing the chromium nickel steel set forth hereinabove and adding to it predetermined 45 amounts of vanadium according to the present invention, the following composition is obtained:

|          | Per cent                     |
|----------|------------------------------|
| Chromium | 6-40                         |
| Nickel   | .5-25                        |
| Carbon   | 0-3                          |
| Vanadium | .2-3                         |
| Iron     | Substantially entire balance |

As exemplary of one successful alloy of useful 55

and advantageous composition, the following may be taken:

|          | Per cent                     |
|----------|------------------------------|
| Chromium | about 18                     |
| Nickel   | about 8                      |
| Carbon   | about .14                    |
| Vanadium | about .5                     |
| Iron     | Substantially entire balance |

10 Such an alloy and hence an article made therefrom is immune from intercrystalline or intergranular disintegration and deterioration and admirably retains its characteristics and properties even in the presence of ordinarily destructive acids, salts and high temperatures, present either singly or together. The properties of the chromium nickel steels themselves, as to ductility and malleability, are not diminished but such properties are influenced and enhanced by the vanadium to give an alloy and article having desirable and admirable properties and characteristics.

15 The vanadium may be incorporated in its isolated elemental state or in the form of one of its salts, compounds, or ores, due allowance being made for the combined or associated elements, and, in each case, a form being selected which introduces no undesirable substance into the alloy.

20 Various modifications in the proportions of the constituents may be made without departing from the spirit and scope of the principles above included.

25 What I claim as new and desire to secure by Letters Patent is:

30 1. Metal articles which in their normal use are subjected to active corrosive influences while the metal in at least a part of the article is in a condition resulting from non-sudden cooling from temperatures within the chromium carbide precipitation range, said articles being resistant to intergranular corrosive attack and being composed of an austenitic chromium-nickel-steel alloy in which the chromium is present to the extent of approximately 18 to 25% and the nickel is present to the extent of approximately 7 to 12%, the balance being principally iron, a small proportion of carbon, and vanadium, the vanadium and carbon being present in the alloy in such proportions and relation to each other that practically the whole of said carbon in said alloy appears therein in stable combination with the vanadium.

35 2. Metal articles which in their normal use are

subjected to active corrosive influences while the metal in at least a part of the article is in a condition resulting from non-sudden cooling of the chromium carbide precipitation range, welding or heating at ranges within the carbide precipitation range without subsequent heating to materially higher temperatures, said articles being resistant to said corrosive attack and being composed of an austenitic chromium-nickel-vanadium-steel alloy in which the chromium is present 10 to the extent of approximately 18 to 25%, the nickel is present to the extent of approximately 7 to 12%, and the vanadium to the extent of approximately 0.5 to 2%, the balance being principally iron with a small proportion of carbon, 15 the vanadium in the alloy being in such proportion with relation to the carbon in the alloy that practically the whole of said carbon in said alloy appears therein in stable combination with the vanadium.

20 3. Metal articles which in their normal use are subjected to active corrosive influences while the metal in at least a part of the article is in a condition resulting from non-sudden cooling within the carbide precipitation range of temperatures, 25 welding or heating within the carbide precipitation range without subsequent heating to materially higher temperatures, said articles being resistant to such corrosive attack and being composed of an austenitic chromium nickel vanadium 30 alloy steel containing approximately 18% chromium, approximately 8% nickel, approximately 0.5% vanadium and not more than about 0.14% carbon, the balance being principally iron and the carbon being substantially all in chemically combined form.

35 4. Metal articles which in their normal use are subjected to active corrosive influences while the metal in at least a part of the article is in a condition resulting from non-sudden cooling within 40 the carbide precipitation range of temperatures, welding or heating within the carbide precipitation range without subsequent heating to materially higher temperatures, said articles being resistant to such corrosive attack and being composed of an austenitic chromium nickel vanadium 45 alloy steel containing approximately 18% chromium, approximately 8% nickel, approximately 0.2-3% vanadium and approximately 0.07-3% carbon, the balance being principally iron and 50 the carbon being substantially all in chemically combined form.

VERE B. BROWNE.